# EUROPEAN PATENT SPECIFICATION

(11) **EP 0 072 175 B1**
(45) Date of publication and mention of the grant of the patent: **08.01.1986**
(21) Application number: 82304080.3
(22) Date of filing: 02.08.1982
(51) Int. Cl.: B22F 7/06

(54) **Method of producing a monolithic alloy component preform**
Verfahren zur Herstellung eines vorgeformten monolitischen Verbundkörpers aus Legierungen
Procédé de fabrication d'une préforme monolithique composite à partir d'alliages

(30) Priority: 07.08.1981 NO 812680
(43) Date of publication of application: 16.02.1983
(73) Proprietor: Mowill, Rolf Jan, N-0386 Oslo 3 (NO)
(72) Inventor: Mowill, Rolf Jan, N-0386 Oslo 3 (NO)
(74) Representative: Jackson, David Spence

## Description

This invention relates to a method of producing a multi-alloy component preform, in which a plurality of powdered alloys are introduced into an outer mold or can having an inner shape corresponding to the outer shape of the desired preform, the main bulk of each powdered alloy being substantially confined to a respective portion of the preform by providing a confining means substantially separating two different alloys and defining an interface therebetween, and consolidating the powdered alloys into a preform.

In highly loaded structures and components, such as gas turbine rotors, the range of properties required very often extend beyond that which is available from a single alloy. As a result of this, various schemes have been proposed and/or tried wherein one component or part is composed of two portions welded, brazed or diffusion bonded together. Generally, however, such methods do not provide the desired bond quality and also often cause a reduction in properties on or near the interface between the two portions.

US-A-3510935 describes a process of manufacturing rod-shaped multilayer semi-finished material in which a block mold is filled with two or more different powders separated by removable partitions. That edge of each partition which is at the bottom during the charging of the powders is serrated, canted or roughened. When each partition is removed, an interlayer is formed with gradual transition between the two different powders which had been separated by the partition. The powders are then compacted and sintered in the block mold.

GB-A-530639 describes a process in which powdered iron or steel is placed in a mold the shape of which corresponds to a part to be made, those parts of the mold in which there are to be hard metal insets or added parts when the article is finished being left free. The iron or steel powder is then covered with a thin plate, a metal foil or a wire fabric, and the remaining part of the mold which corresponds to the hard metal inset or added part is then filled with a mixture of the desired hard metal and an auxiliary metal. Sintering is then carried out with the intermediate plate, foil or fabric combining with the separated metals to form a homogeneous body. Compression is effected before or during the sintering.

According to the present invention the different alloys and properties thereof are utilized in a single component by bringing the alloys together in powder form prior to powder consolidation. Such consolidation may be hot isostatic pressing (HIP), consolidation at atmospheric pressure (CPA) etc.

According to one aspect of the invention, a method of the type defined hereinbefore is characterised in that the confining means has a grid or screen structure to allow a controlled mixing of the powdered alloys through the perforations and a minimum separation of the alloys, eliminating the need for removing the confining means before consolidating the preform.

According to another aspect of the invention a method of the type defined hereinbefore is characterised in that the confining means defines an interface having a large number of protrusions and/or recesses from the general geometric shape of the confining means thereby providing an extended interface and that the material of the confining means is selected so as to provide desired alloy elements to one or both of the alloys adjacent the said interface, thus producing an interface alloy containing the material of the confining means.

The invention will now be described in more detail solely by way of example, with reference to the accompanying drawings, in which:
Fig. 1 is a fragmentary, axial, cross-sectional view of a radial flow turbine wheel preform,
Fig. 2 is a cross-sectional view of the preform illustrated in Fig. 1 along the line II-II thereof,
Fig. 3 is a diagrammatic vertical cross-sectional view of an apparatus for introducing the powdered alloys into the outer mold or can in the production of a disc-shaped preform having concentric alloy portions,
Fig. 4 is a fragmentary cross-sectional view of a mold with an enclosure means or basket defining zig-zag shaped interface,
Fig. 5 is an axial cross-sectional view of a mold with a non-cylindrical basket,
Fig. 6 is a diagrammatic illustration of the typical changes in the outer shape and the interface when producing a final turbine wheel from a preform of the type illustrated in Fig. 1, and
Fig. 7 is a diagrammatical cross-sectional view of a component preform comprising three different powdered alloys.

In Figs. 1 and 2 a radial flow turbine wheel preform 10 is shown to consist of an inner hub portion of alloy B and an outer blade portion in alloy A bonded together into a monolithic component at an interface or rather an interface zone 11.

In Fig. 3 the method of producing such a preform in the form of a cylindrical disc having concentric alloy portion is diagrammatically illustrated. The preform is initially shaped by means of an outer mold or can 12 which the powdered alloys fill. The outer can 12 is positioned in an enclosure 13 placed under vacuum or filled with inert gas to prevent oxidation of the powder particles as well known in the art. To substantially separate the two powders, a confining means in the form of a basket 14 is positioned concentrically within the outer can 12. The two concentric compartments on either side of the basket 14 are filled with the two alloys as indicated. The interface-forming basket 14 may have a grid or screen structure, or it can be made from a perforated sheet, as a zig-zag wall with or without perforations, as a smooth wall etc. The purpose of the basket is one or more of the following:
1) To separate the main bulk of the two alloys.
2) To define the "macro"-geometry of the alloy interface.
3) To allow a controlled mixing of some of the powdered alloy particles in an interface zone on either side of the interface-forming basket to provide an interface zone consisting of an interface alloy compatible with both alloy A and alloy B. Alternatively, such an interface zone may be formed by diffusion of elements of one alloy into the other.
4) To provide a source of alloying elements needed
   a) for the interface alloy as such or
   b) to supply one or more alloying elements to either of the alloys A or B to compensate for depletion of elements caused by diffusion from alloy A to alloy B or vice versa.

The controlled mixing of the powdered alloy particles to provide the interface zone can be obtained by allowing a controlled flow of one powder into the other through the basket 14, when in form of a grid, a screen or the like. For that purpose the filling operation may be controlled so that the rising powder level in one compartment precedes that in the other by a fixed or variable height (h) so that a powder flow from this one to the other compartment can take place above the level in the other compartment with the only restriction being offered by the grid itself. In determining h the specific gravity of the two powders as well as other factors which will influence the behaviour of the flow of powder into the other compartment will have to be taken into account. The height h and/or the restriction offered by the grid can be controlled to vary the amount of mixing of one alloy into the other and/ or the thickness of the resulting interface zone. Variation of the latter can be used to compensate for interface zone slimming during subsequent forging of the preform. The controlled transfer of portions of one powdered alloy into the adjacent layer of the other powdered alloy can also be achieved in other ways, for instance by rotating the inner basket 14 or even rotating the basket as well as the outer can 12 using the centrifugal force to provide said controlled transfer. Shaking would be a further alternative. Instead of transferring powder particles, merely one or more elements of one alloy may be transferred across the interface to form an interface zone, and this may be accomplished by diffusion when the basket 14 has been removed prior to or during the consolidation step or possible further metallurgical treatment.

A zig-zag type basket as shown in Fig. 4 would provide a considerable interface zone by diffusion alone.

The basket 14 may be removed by decomposing or melting the material in the basket whereupon the molten or decomposed material is extracted and/or evaporated. However, as mentioned above, the material may also be incorporated in one or both of the alloys A or B or in the interface alloy.

Both the basket 14 and the outer can 12 may have different shapes in order to give the best final outer shape and interface configuration as illustrated in Fig. 5 for the basket 14.

After the powder preform has been consolidated, for example by hot isostatic pressing, it may be subjected to superplastic or hot die forging in which the material will flow into its near net shape. The turbine wheel blank would then be ready for heat treatment and final machining. Hot isostatic pressing may be used to shape the preform to final near net shape instead of merely for consolidation purposes.

The method described will provide a sound monolithic structure without the many uncertain aspects connected with diffusion bonding of solid parts. Also, the interface alloy will provide a compliance zone between the two alloys which for example could have a coefficient of expansion between those of the alloys A and B after the powder preform has been consolidated. A pressing and/or forging operation can follow which will give final dimensions prior to machining, as shown as an example in Fig. 6, in which the interface is indicated at 11 before forging and at 15 after forging. The outer contour of the preform is indicated at 16 and that of the final turbine wheel at 17. The line 16' indicates the contour between the blade and the hub portion of the turbine wheel. Trial and error methods will have to be used to determine the interface configuration 11 in the preform 10 which will result in the desired interface configuration 15 in the final component. The interface alloy now has properties which lies between those of A and B. Thus, there is no sharp "bonding line" between the two alloys.

A preform according to the invention can consist of more than two alloys and more than one basket 14. Also, a basket can be pre-loaded with powder prior to inserting the basket into the outer can. This is illustrated in Fig. 7, in which a basket 14' preloaded with powdered alloy B and a basket 14" preloaded with powdered alloy C may be placed into the outer can 12, whereupon a powdered alloy A may be introduced to fill the remaining space between the two baskets. In this instance, the baskets would have an internal air tight seal 18 of a material which would easily be decomposed and may be extracted or absorbed into the powder on either side of the basket when exposed to the operation temperature of the consolidation process or to other influences.

In the example in Fig. 7 material C could be an alloy which is resistant to corrosion and abrasion at high temperature, whereas the requirement for high ultimate tensile strength is less than for the alloys A and B. The alloy B would be the alloy of the highest tensile strength. The properties of alloy A would fall between those of alloys B and C.

The method of the invention has the potential of giving turbines the ability to operate at very high temperatures and tip-speeds without incurring risk of failure by inadequate and unreliable bonding. The method offers numerous interface geometry choices for the optimization of the structural properties of the finished turbines.

In the specification the term "alloy" should be taken to refer to any solid, structural composition composed of two or more chemical elements of which at least one is a metal, providing this composition lends itself to powder metallurgy processing methods including consolidation steps. Thus, not only mixtures of elemental metals, but also compositions such as metal carbides and ceramic materials are comprised by the term "alloy" as used in the present Specification.

## Claims

1. A method of producing a multi-alloy component preform, in which a plurality of powdered alloys are introduced into an outer mold or can (12) having an inner shape corresponding to the outer shape of the desired preform, the main bulk of each powdered alloy being substantially confined to a respective portion of the preform by providing a confining means (14) substantially separating two different alloys and defining an interface therebetween, and consolidating the powdered alloys into a preform, characterized in that the confining means (14) has a grid or screen structure to allow a controlled mixing of the powdered alloys through the perforations and a minimum separation of the alloys, eliminating the need for removing the confining means before consolidating the preform.

2. A method of producing a multi-alloy component preform, in which a plurality of powdered alloys are introduced into an outer mold or can (12) having an inner shape corresponding to the outer shape of the desired preform, the main bulk of each powdered alloy being substantially confined to a respective portion of the preform by providing a confining means (14) substantially separating two different alloys and defining an interface therebetween, and consolidating the powdered alloys to a preform, characterised in that the confining means (14) defines an interface having a large number of protrusions and/or recesses from the general geometric shape of the confining means thereby providing an extended interface, and that the material of the confining means (14) is selected so as to provide desired alloy elements to one or both of the alloys adjacent the said interface, thus producing an interface alloy containing the material of the confining means (14).

## Revendications

1. Procédé de fabrication d'une préforme en composants en alliages multiples, selon lequel on introduit plusieurs alliages en poudre dans un moule ou boîte exterieur (12) ayant une forme intérieure qui correspond à la forme extérieure de la préforme désirée, la mass principale de chaque alliage en poudre étant pratiquement confinée à une partie respective de la préforme par l'établissement d'un moyen de confinement (14) qui sépare sensiblement deux alliages différents et définit une interface entre eux, et de consolidation des alliages pulvérulents en une préforme, caractérisé en ce que le moyen de confinement (14) présente une structure en grille ou en tamis pour permettre un mélange réglé des alliages en poudre à travers les perforations et un minimum de séparation des alliages, en éliminant la nécessité d'enlever le moyen de confinement avant de consolider la préforme.

2. Procédé de fabrication d'une préforme en composants en alliages multiples, selon lequel on introduit plusieurs alliages en poudre dans un moule ou boîte exterieur (12) ayant une forme intérieure qui correspond à la forme extérieure de la préforme désirée, la masse principale de chaque alliage en poudre étant pratiquement confinée à une partie respective de la préforme par l'établissement d'un moyen de confinement (14) qui sépare sensiblement deux alliages différents et définit une interface entre eux, et de consolidation des alliages pulvérulents en une préforme, caractérisé en ce que le moyen de confinement (14) définit une interface présentant un grand nombre de protubérances et/ou d'évidements à partir de la forme géométrique générale du moyen de confinement pour obtenir ainsi une interface prolongée et en ce que le matériau du moyen de confinement (14) est choisi de manière à fournir les éléments désirés d'alliage à l'un ou aux deux alliages adjacentes à ladite interface, en produisant ainsi un alliage interface qui contient la matière du moyen de confinement (14).

## Patentansprüche

1. Verfahren zur Herstellung eines Vorformlings bzw. Rohlings aus einer Mehrfachlegierung, bei dem mehrere pulverförmige Legierungen jeweils in eine äußere Form bzw. ein äußeres Behältnis (12) eingefüllt werden, wobei das Behältnis eine Innenform aufweist, die der äußeren Form des gewünschten Vorformlings entspricht, und wobei die Hauptmenge jeder pulverförmigen Legierung im wesentlichen einem entsprechenden Teil des Vorformlings zugeordnet wird, indem ein Trennelement (14) vorgesehen wird, daß zwei verschiedene Legierungen im wesentlichen voneinander trennt und eine Grenzfläche zwischen den Legierungen definiert, und bei dem die Legierungen zu dem Vorformling verfestigt werden, dadurch gekennzeichnet daß das Trennelement (14) eine Gitter- oder Siebstruktur aufweist, um eine kontrollierte bzw. gesteuerte Vermischung der pulverisierten Legierungen durch die Perforation hindurch und eine minimale Separation der Legierungen zu ermöglichen, derart, daß das Erfordernis der Entfernung des Trennelements vor Verfestigung des Vorformlings entfällt.

2. Verfahren zur Herstellung eines Vorformlings bzw. Rohlings aus einer Mehrfachlegierung, bei dem mehrere pulverförmige Legierungen jeweils in eine äußere Form bzw. ein äußeres Behältnis (12) eingefüllt werden, wobei das Behältnis eine Innenform aufweist, die der aüußeren Form des gewünschten Vorformlings entspricht, und wobei die Hauptmenge jeder pulverförmigen Legierung im wesentlichen einem entsprechenden Teil des Vorformlings zugeordnet wird, indem ein Trennelement (14) vorgesehen wird, das zwei verschiedene Legierungen im wesentlichen voneinander trennt und eine Grenzfläche zwischen den Legierungen definiert, und bei dem die Legierungen zu dem Vorformling verfestigt werden, dadurch gekennzeichnet, daß das Trennelement (14) eine Grenzfläche definiert mit einer großen Zahl von Vorsprüngen und/oder Ausnehmungen entsprechend der Geometrie bzw. Struktur des Trennelements, wodurch eine vergrößerte Grenzfläche erhalten wird, und daß das Material des Trennelements (14) so ausgewählt ist, daß es ein gewünschtes Legierungselement für die eine oder beide Legierungen darstellt, die an der Grenzfläche angrenzen, so daß eine Grenzschichtlegierung entsteht, die das Material des Trennelements (14) enthält.
